

## UNITED STATES PATENT OFFICE

2,118,055

## COATINGS ON ALUMINUM

James W. Newsome, New Kensington, Pa., assignor to Aluminum Company of America, Pittsburgh, Pa., a corporation of Pennsylvania

No Drawing. Application June 22, 1937,  
Serial No. 149,680

8 Claims. (Cl. 148—6)

This invention relates to the production of oxide-coated aluminum surfaces, and it is particularly concerned with a method for the production of a substantially colorless, hard, adherent and adsorptive coating consisting substantially of aluminum oxide on an aluminum surface by chemical treatment without the external application of electric current. The term aluminum as used herein and in the appended claims is intended to include both aluminum in its various degrees of purity and the aluminum base alloys.

Oxide coatings have found extensive application for the protection and decoration of aluminum surfaces. This field has been extended particularly in recent years as a result of the development of the so-called anodic oxidation methods in which hard, adherent, abrasion-resistant coatings are formed on aluminum by electrolytic oxidation. These coatings are generally more or less porous and adsorbent, and can be colored, impregnated with corrosion-inhibiting substances, sealed, or otherwise treated, as their particular use demands. However, these methods do not lend themselves readily to the production of oxide coatings on small articles, such as buttons, eyelets, and the like, and their use is not economical in the production of certain types of articles intended for sale at relatively low prices.

While it has been recognized that the methods of producing coatings on aluminum by simple chemical treatment without the application of electrical energy would be desirable for use in the coating of small articles, the methods heretofore available, and known to the art, for providing oxide coatings on aluminum by a simple chemical treatment have not produced coatings which have a suitable combination of properties to recommend them for general use. In order to be satisfactory for general use, it is desirable that the coating produced should be sufficiently hard and adherent to resist the abrasion incident to ordinary use, and should preferably be substantially colorless and more or less adsorbent, so that it can be colored by dyeing or pigmenting.

It is an object of this invention to provide a chemical treatment method for the production of an oxide coating on aluminum having a combination of properties permitting its general use as a finishing coating. It is more particularly an object of this invention to provide a method for the production of a hard, adherent, adsorbent and substantially colorless coating comprising aluminum oxide on an aluminum surface by simple chemical treatment without the aid of an electric current.

It is a further object of this invention to provide a coating of the above nature and properties which is resistant to abrasion and corrosion, and which is free from pits and discolorations frequently encountered with former chemical coatings applied by the usual chemical treatments. It is a still further object of the invention to provide a chemical coating bath which may be used continuously over a relatively extended period of time while continuing to maintain equilibrium conditions of reagent concentration, so that it functions uniformly over the term of its use.

I have discovered that improved coatings of the type described hereinabove can be produced on aluminum and aluminum alloy surfaces by treatment of the said surfaces with a solution containing an alkali metal salt of an organic hydroxy acid and an alkali metal aluminate. The treatment is preferably carried out in a sodium aluminate solution containing a substance of the group composed of sodium glycolate, sodium lactate, sodium tartrate, sodium citrate, sodium malate, sodium salicylate, and sodium para hydroxy benzoate. The article to be coated is preferably immersed in the solution at an elevated temperature. The reaction between the coating solution and the metal surface, which is at first fairly vigorous, gradually becomes slower and finally practically stops, generally within twenty to thirty minutes when operated at temperatures of from 85 to 95° centigrade. The coating produced is relatively hard, adherent, abrasion-resistant and corrosion-resistant, and is relatively free from pits and streaks. It is more or less adsorbent and substantially colorless.

Satisfactory solutions may be obtained by using aluminate solutions containing as little as 0.1 per cent of sodium aluminate or as much as 2.0 per cent, but for most purposes a concentration of 0.5 to 1.0 per cent has proved most satisfactory. The amount of the salt of the organic hydroxy acid may vary somewhat depending on the particular salt used. In general, when the sodium salts are used, amounts ranging from about 0.025 per cent to 1.5 per cent have proved satisfactory. With the sodium salts of glycollic, lactic, tartaric, citric, malic, and para hydroxy benzoic acids, I have found it preferable to use a solution in which the ratio of the sodium salt of the organic hydroxy acid to the sodium aluminate is from about 1:1 to 2:1, and I prefer in most cases to use a solution containing 0.5 to 1.0 per cent of the salt of the organic hydroxy acid and 0.5 per cent of sodium aluminate. The sodium salicylate seems to be more effective, and it is desirable to

use only about 0.25 per cent of sodium salicylate with from 0.5 to 1.0 per cent of sodium aluminate, or in a ratio of about one part salicylate to 2 to 4 parts aluminate. It is preferred first to make up an aqueous solution of the salt of the organic hydroxy acid and then add the alkali metal aluminate. When the aluminum or aluminum alloy article is immersed in the solution, preferably between 85 and 95° C. as aforesaid, the solution rapidly attains equilibrium conditions, and any excess of alumina caused by the action of the bath in producing the oxide coating precipitates out and settles at the bottom of the container.

Preliminary cleaning of the aluminum surface to be coated is not essential, though it may be desirable. I have found that aluminum surfaces on which there is a film of oil may be satisfactorily coated when treated according to my invention, without any preliminary treatment to remove the grease. It is generally preferred, however, to use a clean aluminum surface. In some cases it may be preferred to preliminarily etch the surface to be coated. Particularly good results may be produced on surfaces preliminarily etched in hydrofluoric acid, followed by washing with strong nitric acid.

The properties of the coating obtained by the method of my invention will vary somewhat with the composition of the aluminum or aluminum alloy surface treated, and the exact conditions of treatment used. Certain aluminum alloys, by reason of the presence of elements such as iron, manganese, or copper, have a tendency to develop coloration in the coatings produced, and in such cases the use of somewhat weaker solutions than those noted in the preferred solutions above referred to may be desirable. Although the preferred temperature range has been stated as between 85 and 95° C., it may vary from room temperature to the boiling point. The time required to produce a coating of the required thickness at the lower temperature must, of course, be lengthened in such instance, and at room temperature from 10 to 20 hours may be required.

As a specific example of the method of coating aluminum according to the process of my invention, I may cite the following. The aluminum to be coated was immersed in a solution containing 1.0 per cent sodium aluminate and 1.0 per cent sodium tartrate. The solution was maintained at a temperature of 85° C., and the treatment continued for a period of about 30 minutes. After treatment the aluminum was found to be coated with a hard, adherent coating having an average thickness, as determined by microscopic examination of a cross section, of about 0.00008 inch. This coating was substantially colorless, and was hard, abrasion-resistant and of good corrosion resistance.

I claim:

1. A method of producing a substantially col-

orless protective coating on an aluminum surface, comprising treating said surface with a solution containing an alkali metal salt of an organic hydroxy acid and an alkali metal aluminate.

2. A method of producing a substantially colorless protective coating on an aluminum surface, comprising treating said surface with a solution containing an alkali metal salt of an organic hydroxy acid and an alkali metal aluminate at a temperature of 85° to 95° centigrade.

3. A method of producing a substantially colorless protective coating on an aluminum surface, comprising treating said surface with a solution containing an alkali metal aluminate and 0.025 to 1.5 per cent of a sodium salt of an organic hydroxy acid selected from the group consisting of glycollic acid, lactic acid, tartaric acid, citric acid, malic acid, salicylic acid, and para hydroxy benzoic acid.

4. A method of producing a substantially colorless protective coating on an aluminum surface, comprising treating said surface with a solution containing from 0.1 to 2.0 per cent of sodium aluminate and a sodium salt of an organic hydroxy acid selected from the group consisting of glycollic acid, lactic acid, tartaric acid, citric acid, malic acid, salicylic acid and para hydroxy benzoic acid.

5. A method of producing a substantially colorless protective coating on an aluminum surface, comprising treating said surface with a solution containing from 0.1 to 2.0 per cent of sodium aluminate and a sodium salt of an organic hydroxy acid selected from the group consisting of glycollic acid, lactic acid, tartaric acid, citric acid, malic acid, and para hydroxy benzoic acid in which the ratio of the sodium salt of the organic hydroxy acid to the sodium aluminate is from about 1:1 to 2:1.

6. A method of producing a substantially colorless protective coating on an aluminum surface, comprising treating said surface with a solution containing about 0.5 per cent of sodium aluminate and 0.5 to 1.0 per cent of a salt of an organic hydroxy acid selected from the group of hydroxy acids consisting of glycollic acid, lactic acid, tartaric acid, citric acid, malic acid, and para hydroxy benzoic acid.

7. A method of producing a substantially colorless protective coating on an aluminum surface, comprising treating said surface with a solution containing sodium aluminate and sodium salicylate in a ratio of about one part of salicylate to 2 to 4 parts aluminate.

8. A method of producing a substantially colorless protective coating on an aluminum surface, comprising treating said surface with a solution containing about 0.25 per cent of sodium salicylate and 0.5 to 1.0 per cent of sodium aluminate.

JAMES W. NEWSOME.